

Patented July 11, 1950

2,514,901

# UNITED STATES PATENT OFFICE

2,514,901

## BITUMINOUS EMULSIONS FOR TREATMENT OF COAL AND METHODS OF PREPARING SAME

Charles R. Roseneranse, Pittsburg, Kans., assignor  
of fifty per cent to Joe F. Klaner, Jr., Pittsburg,  
Kans.

No Drawing. Application November 17, 1948,  
Serial No. 60,634

8 Claims. (Cl. 106—277)

1

This invention relates to a colloidal suspension to be sprayed on coal to form a permanent coating rendering the coal substantially dust-proof and impervious to moisture and oxidation, the present subject matter involving an improvement over the subject matter in my Patent No. 2,431,891, issued December 2, 1947.

An important object of this invention is to provide a colloidal suspension which does not require the application of heat when it is sprayed or coated on coal, and which while forming a hard, dry, and permanent coating on the coal, does not cause the coal particles to objectionably adhere together.

Another important object of the invention is to provide a bituminous emulsion for coating coal which although of microscopic thinness, positively seals the coal permanently against weathering and slacking during ordinary handling and storage of the coal.

Another important object of the invention is to provide a bituminous coating for coal which can be removed only by combustion or immersion of the coal in a suitable solvent other than water, and which as a result renders the coal clean to handle and non-soiling with respect to other objects or materials with which the coated coal may come into contact.

By "coal" as referred to herein, is meant bituminous, semi-bituminous, anthracite, semi-anthracite, or the so-called lignite coals, and others comprehended by these terms.

After extensive experimentation with the process and composition disclosed in the patent mentioned hereinabove, I have discovered that a number of improvements could be made wherein the resulting emulsion produces a better sheen and color on the coal treated, affords better protection to the coal, and produces an odorless coating for the coal.

The primary improvement resides in the substitution of coal tar pitch for the asphalt, artificial or natural, employed in the patented process. As is well known in the art, coal tar pitch is the residue from the distillation of coal tar from which the aromatic substances have been removed. Coal tar pitch is a solid substance of varying degrees of hardness which is determined by the amount of distillation used to remove the aromatic substances. In the dry state it has an approximate specific gravity of 1.20.

Since coal tar pitch is less soluble than asphalt, obviously coal coated with coal tar pitch will be better protected against moisture and oxidation. Also, coal coated with coal tar pitch is relatively

2

odorless as compared to coal coated with asphalt emulsion. To the best of the applicant's knowledge, coal tar pitch has never before been successfully employed in manufacturing an emulsion for the treatment of coal because of the acidity of the pitch. The herein described improved process and composition includes a novel method of reducing this objectionable acidity.

In the patented process before the asphalt is run through the colloid mill for admixture with the aqueous dispersion, it was found necessary to use an asphalt having an initial penetration of 8 to 10 mm. and preferably a ductility rating of about 15 to 18 mm. and then blowing the asphalt at an oxidizing temperature in an oxidizing chamber with about 4,000 cubic feet of air per minute for a length of time necessary to reduce the penetration of the asphalt to about 2.6 to 3.0 mm. thereby raising the melting point of the asphalt to about 210 to 260 degrees F. While the same treatment can be applied to coal tar pitch with advantageous results, it has been found herein that no such treatment is required when a coal tar pitch having a penetration from 26 to 30 mm. and a melting point of from 190 to 210 degrees F. is employed.

In the patented process it was also necessary to simultaneously run the heated and treated asphalt together with the heated aqueous dispersion through a colloid mill operating at substantially 5,000 R. P. M. and at a constant rate. A marked advantage is obtained by running the colloid mill at approximately half its normal rate of speed.

It has been found that by reducing the amount of material entering the colloid mill instead of reducing the speed of the mill itself, a marked improvement of the resulting emulsion is obtained with respect to the stability of the emulsion. In other words, rather than reduce the speed of the colloid mill by one-half, the material is fed into the mill at a rate equal approximately to one-half of the flow or output capacity of the mill.

In the patented process, also, an aqueous dispersion was employed containing a number of essential ingredients. The applicant has found that a variation of the percentages by weight of these ingredients produces a dispersion which allows the substitution of coal tar pitch for asphalt and which also permits him to dispense with the blowing or pre-treatment of both the asphalt and the coal tar pitch.

Moreover, the applicant has found that a prior mixture in a mixing chamber of the heated asphalt and coal tar pitch with the aqueous dis-

persion prior to running the suspension or mixture into the colloid mill produces a superior and more stable emulsion as an end product.

At this point the improved process and composition will be described in detail. As a starting material, asphalt, natural or artificial, or coal tar pitch may be employed provided the penetration is in the range of 2.6 to 30.0 mm. and the melting point is between 190 and 260 degrees F., the preferred embodiment being coal tar pitch. When employing asphalt, a material having a penetration of 2.6 mm. is preferred and if an asphalt having a higher penetration is employed it will be found advantageous to reduce the penetration and raise the melting point thereof by 15 the oxidation and blowing treatment fully described in the patented process. If a coal tar pitch having a penetration of from 26 to 30 mm. and a melting point of from 190 to 210 degrees F. is employed, no pre-treatment such as blowing or oxidation is required.

The coal tar pitch is then heated in a container until it is fluid, that is, to a temperature not exceeding 300 degrees F., and then run preferably into a mixing chamber where it is mixed with preferably an equal volume of an aqueous dispersion to be described hereinafter. Thereafter the admixture or suspension of the pitch and the dispersion is run into a colloid mill at a velocity equal approximately to one-half of the flow capacity of the colloid mill. That is, if the capacity of the colloid mill is 4,000 gallons per hour, the speed of the pumps which introduce the suspension into the mill is reduced so that the mill can only produce 2,000 gallons per hour.

The liquid phase of the emulsion or what may be termed the aqueous dispersion comprises the following ingredients:

|                | Per cent by weight |
|----------------|--------------------|
| Water          | 93.74-95.04        |
| Resin          | 3.00               |
| Bentonite clay | 1.40-1.60          |
| Tall oil       | 0.10               |
| Caustic soda   | 0.46-1.56          |

The resin employed in the above formulation is a substantially petroleum hydrocarbon insoluble pine wood resin such as described in the Patent No. 2,193,026, issued March 2, 1940, to Lucius Coleman Hall.

The ingredient tall oil is described in the Patent No. 2,305,498, issued December 14, 1942, to Ernest Segesemann and is well known in the art.

The preferred embodiment of the above dispersion for use especially with coal tar pitch in the above improved process is as follows:

|                | Per cent by weight |
|----------------|--------------------|
| Water          | 93.74              |
| Resin          | 3.00               |
| Bentonite clay | 1.60               |
| Tall oil       | 0.10               |
| Caustic soda   | 1.56               |

It will be noted that the dispersion mentioned immediately hereinabove differs from the one disclosed in the Patent 2,431,891 in that the amount of bentonite clay and caustic soda is increased. The increased bentonite content improves the stability of the emulsion and the increased amount of caustic soda neutralizes the acidity in the coal tar pitch, which acidity was responsible for the prior inability of providing a stable emulsion from bituminous material such as coal tar pitch.

It has also been found that a prior treatment of the coal tar pitch when heated to a state of fluidity before admixture with the aqueous dispersion improves the stability of the emulsion and the coating properties thereof. This prior treatment includes the addition of a weak solution of caustic soda in glycerine to the fluid coal tar pitch. The preferred amount of caustic soda to be added to the coal tar pitch is 0.44% by weight of the caustic soda to the weight of the coal tar pitch. This solution of caustic soda and glycerine is, of course, thoroughly mixed throughout the fluid coal tar pitch phase.

Thus it will be seen that a novel process and composition is provided for coating coal whereby the latter will be rendered impervious to moisture, oxidation, etc. The coating material of the present invention, requiring no heating above its freezing point, can be sprayed or atomized on the coal, directly from the storage containers, and by means of any suitable spraying equipment. The bituminous emulsion provided by the improved process hereinabove described produces a better sheen and color on the coal, affords better protection to the coal because of the lesser solubility of coal tar pitch as compared to asphalt, and produces a relatively odorless coating for the coal.

While a preferred embodiment of the applicant's process and composition has been described hereinafter, it will be readily understood that minor variations in the process and composition may be made by those skilled in the art without departing from the spirit of the invention and the scope of the appended claims.

Having described the invention, what is claimed as new is:

1. The method of making a colloidal suspension for spraying on coal at atmospheric temperature to form a permanent coating rendering the coal substantially dust-proof and impervious to moisture and oxidation, comprising heating coal tar pitch having a penetration of 2.6 to 30.0 mm. and a melting point of 190° to 260° F. to a temperature not over 300° F., running the heated coal tar pitch through a mixing chamber together with an aqueous dispersion heated to about 180° F., then simultaneously running the suspension through a colloid mill at a velocity equal approximately to one-half of the flow capacity of the mill, said dispersion comprising by weight substantially 93.74-95.04% water, 3.00% of a substantially petroleum hydrocarbon insoluble pine wood resin, 1.40-1.60% bentonite, 0.10% tall oil, and 0.46-1.56% caustic soda, then rapidly reducing the resultant emulsion to a temperature of 150° F. for storage.

2. The process of claim 1, and the step of adding to the heated coal tar pitch prior to admixture with the dispersion a relatively weak solution of caustic soda in glycerine.

3. The process of claim 2, wherein the caustic soda is added in an amount equal to 0.44% by weight of the coal tar pitch.

4. The method of making a colloidal suspension for spraying on coal at atmospheric temperature to form a permanent coating rendering the coal substantially dust-proof and impervious to moisture and oxidation, comprising heating to a temperature not over 300° F., coal tar pitch having a penetration of 26-30 mm. and a melting point of 190°-210° F., running the heated pitch through a mixing chamber together with an aqueous dispersion heated to about 180° F., then simultaneously running the suspension through a

colloid mill at a velocity equal approximately to one-half of the flow capacity of the mill, said dispersion comprising by weight substantially 93.74% water, 3.00% of a substantially petroleum hydrocarbon insoluble pine wood resin, 1.60% bentonite, 0.10% tall oil, and 1.56% caustic soda, then rapidly reducing the resultant emulsion to a temperature of 150° F. for storage.

5. The process of claim 4, and the step of adding to the heated coal tar pitch prior to admixture with the dispersion a relatively weak solution of caustic soda in glycerine.

6. The process of claim 5, wherein the caustic soda is added in an amount equal to 0.44% by weight of the coal tar pitch.

7. The method of making a colloidal suspension for spraying on coal at atmospheric temperature to form a permanent coating rendering the coal substantially dust-proof and impervious to moisture and oxidation, comprising heating to a temperature not over 300° F., coal tar pitch having a penetration of 26-30 mm. and a melting point of 190°-210° F., simultaneously running the heated pitch through a colloid mill together with an aqueous dispersion heated to about 180° F., said dispersion containing by weight substantially 95.04% of water, 3% of a substantially petroleum hydrocarbon insoluble pine wood resin, 1.4% of bentonite, 0.10% of tall oil, and 0.46% of caustic soda, then rapidly reducing the

temperature of the resultant emulsion to about 150° F., for storage.

8. A colloidal suspension for spraying on coal at atmospheric temperature to form a permanent coating rendering the coal substantially dust-proof and impervious to moisture and oxidation, comprising coal tar pitch having a penetration of 26-30 mm. and a melting point of 190°-210° F. which has been simultaneously run through a colloid mill together with an aqueous dispersion heated to about 180° F. at a velocity equal approximately to one-half of the flow capacity of the mill, said dispersion comprising by weight substantially 93.74% water, 3.00% of a substantially petroleum hydrocarbon insoluble pine wood resin, 1.60% bentonite, 0.10% tall oil, and 1.56% caustic soda.

CHARLES R. ROSENCRANSE.

#### REFERENCES CITED

The following references are of record in the file of this patent:

#### UNITED STATES PATENTS

| Number    | Name        | Date          |
|-----------|-------------|---------------|
| 1,807,808 | Symons      | June 2, 1931  |
| 2,190,034 | Levin       | Feb. 13, 1940 |
| 2,431,891 | Rosencranse | Dec. 2, 1947  |

#### FOREIGN PATENTS

| Number  | Country       | Date         |
|---------|---------------|--------------|
| 462,111 | Great Britain | Mar. 2, 1937 |